

1

2,926,115

## CORK RECOVERY

William G. Van Beckum, Sam Mateo, and Robert W. Miller, Scotia, Calif., assignors to The Pacific Lumber Company, San Francisco, Calif., a corporation of Maine

No Drawing. Application August 30, 1956  
Serial No. 606,974

6 Claims. (Cl. 162—21)

This invention relates to the treatment of cork-containing, woody material to separate the cork from the non-cork material. More particularly this invention relates to recovery of cork from bark containing cork mixed with fibrous material.

Commercial supplies of cork, both today and since the inception of the cork industry, have come almost exclusively from the cork oak, *Quercus suber*. Commercial stands of that species of oak are limited almost entirely to an area bordering on the Mediterranean. The great majority of commercial cork comes from Spain, Portugal and North Africa.

Cork is the outer bark of the cork oak, i.e., the dead part of the bark overlying the inner living bark. This outer layer is stripped from time to time. After suitable processing, such as sorting into grades and boiling, it passes into channels of trade.

There exist many uses of cork all of which depend upon some one or more of the properties of the material. These properties include a high degree of buoyancy, a high degree of compressibility without lateral spreading, a high resilience, resistance to moisture and liquid penetration, a high coefficient of friction, a low thermal conductivity, a high ability to absorb mechanical and acoustical vibrations and a high degree of stability and resistance to deterioration.

Thus bottle stoppers (the "corks" of common parlance) rely upon resilience, compressibility and resistance to liquid penetration. Cork insulation, which is made by grinding cork to small particle size and bonding the particles together by heat and pressure, utilizes the low thermal conductivity of cork. Composition cork is made by similarly grinding cork into small particles which, however, are bonded together by added adhesive. It has many uses such as gaskets, liners for crown top bottle stoppers, inner soles of shoes, etc. Mere mention of these uses will bring to mind the qualities of cork which make that material so versatile and useful. Another use of cork is in linoleum, wherein linseed oil is used to impregnate very finely divided cork known as cork flour.

In all its uses the cellular character of cork is a property of prime importance. In the aging of the outer bark of the cork oak a cellular structure is produced in which tetrakidecahedral (14-sided) cells are packed closely together with virtually no interstices (other than macro interstices produced by cracking and splitting) and with each cell consisting of a volume of air entrapped by a tough wall. It is this remarkable cellular structure which imparts to cork its many useful properties.

The literature on the subject of cork indicates that all cork of any consequence comes from *Quercus suber* grown in the Mediterranean area; that the transplanted species, i.e., trees planted in other parts of the world, are of no commercial consequence; and that other species of cork-bearing trees have been, at best, minor sources of an inferior product. The prevailing view is summed up by Faubel in "Cork and the American Cork Industry,"

2

published by Cork Institute of America, rev. ed., page 1, as follows:

"For reasons which Nature alone controls, this oak tree grows in commercial stands only in areas bordering the Mediterranean Sea and all attempts to establish cork forests in this country and elsewhere have thus far been unsuccessful."

Such authorities as Faubel fail even to mention the known fact that cork exists in large proportion combined with fibrous and amorphous material in the bark of other trees, such as Douglas fir. The lack of commercial methods for separating the cellular cork from the fibrous and amorphous material in such barks explains the fact that, by and large, the literature on cork does not even mention cork-bearing Douglas fir bark and the like as a potential source of cork.

It is a known fact (cf. Kurth in Journal Forest Products Research Society, vol. 1, pp. 98-103 (1951)), that Douglas fir bark contains 25 to 50% cork. In TAPPI, 20 vol. 35, No. 2, February 1952, it is stated that cork may occur in the bark of the lower parts of mature Douglas fir trees in amounts exceeding 50%.

Douglas fir bark and other cork-containing barks are stripped from saw, pulp and other logs in vast quantities 25 and are a potential source of very large amounts of cork. Work has been done on the recovery of cork from such barks, as described in more detail below, but by and large these barks have very limited value being used, for example, largely as fuels.

Previous efforts to separate cork from noncork material in bark have employed mechanical attrition, such as ball milling or hammer milling. By such means it is supposed that the fibrous material, being more friable when in somewhat dry condition than the cork, would disintegrate to a greater degree than the cork. The object of these prior methods has been to separate the fibrous and amorphous noncork material as fine particles, and to selectively concentrate the cork in the coarser particles.

Whatever the merits of mechanical attrition, it is defective in practice because, among other things, the cork particles are flattened and compacted and are substantially reduced in size and resiliency by the impact of the milling elements. These reductions are serious deterrents to the quality of cork.

It is an object of the invention to provide an improved method of separating cork from noncork materials in natural products such as bark.

It is another object of the present invention to provide a method of separating cork from noncork material in natural products, particularly bark, such method being of a nature that it does a minimum of damage to the porous, cellular character of the cork and in fact, in some important respects improves it.

It is a particular object of the invention to provide a method of treating Douglas fir bark to obtain fractions thereof which are high in cork content, such method avoiding the necessity and disadvantages of milling operations.

These and other objects of the invention will be apparent from the ensuing description and the appended claims.

In accordance with the invention, a natural product such as bark, e.g., Douglas fir bark is selected which contains corky and noncorky material, the latter being usually of a fibrous and amorphous character. Such product is reduced to a suitable size for handling, if that is necessary, by shredding, cutting or the like. It is then subjected to the action of steam at high pressure and temperature. The steam pressure is then suddenly released to disintegrate the brash, amorphous noncork particles of the bark by reason of the explosive force of the expanding steam.

On the other hand, the softer cork layers in the bark are only softened further as a result of the steaming treatment and are only moderately reduced in size. Furthermore resiliency of the cork particles to some extent is actually improved as a result of the "puffing" action of the steam treatment.

This operation may be carried out in any suitable apparatus, for example, in a so-called "Masonite" gun, such as used to fiberize wood chips for production of hard board. Such apparatus is well known in the lumber and wood products industries, and it requires no detailed description herein. It consists essentially of a chamber with inlet means to introduce steam under pressure and an outlet which can be opened to blow out the chips after they have been processed sufficiently within the chamber by means of high pressure steam.

The steam pressure and temperature, and the duration of the processing or "cooking" operation may vary considerably, as will be apparent from the examples below. If conditions are not adequately severe, that is, if too low a pressure and temperature and/or too short a "cooking" period is employed, the essential disintegrating effect of the steam is not obtained. On the other hand, if conditions are too severe, that is, if too high a pressure and temperature and/or too long a cooking period are employed, then it will be found that the steam disintegrates and causes excessive deterioration of the cork material, as well as the noncork material. From the description and teachings contained herein, and with a modicum of trial and error, conditions of pressure, temperature, and time can be readily found to obtain optimum or approximately optimum results.

After the cooking step has been completed and the mass of cooked product has been expelled or blown from the cooking chamber, the cooked product can be dried by any suitable means, preferably by countercurrent contact with a current of hot air. The dried, cooked product consists of a mass of disintegrated fibrous and amorphous material which is predominantly small in particle size, together with corky material which will also have been disintegrated or reduced in size but not nearly to the same degree as the noncork material. Moreover, this corky material preserves substantially intact its original porous cellular character and it constitutes an excellent material for insulation. The corky material is readily separated from the fibrous and amorphous, noncork material by size classification, as by passing through a series of screens of diminishing size. It will be found that the percentage of cork in the coarser fractions is much greater than in the original product, and that the percentage of fibrous material is much greater in the finer fractions. Such size classification or screening may be carried out repeatedly, as by taking a given fraction and subjecting it to a second screening. Also, the coarsest fractions, e.g.,  $+\frac{3}{8}$ " material and if desired the  $-\frac{3}{8}$ " +8 mesh fraction may be recycled, i.e., given a second cooking step, preferably under milder conditions.

Steam is the preferred medium for cooking and selectively disintegrating woody material, and it is preferably injected into the cooking chamber directly from a boiler. However, steam may be generated in situ, as by means

of heating moist woody material by any suitable means, for example, hot air, or by means of efficient heat transfer from heated elements, such as fins. Steam pressures of about 200 to 600 p.s.i. and cooking periods of about 30 to 90 seconds may be employed, although greater and lesser pressures and cooking periods may be employed depending upon the bark, its moisture content and other factors. Also, hot combustion gases may be employed instead of steam as a source of heat, relying upon the moisture in the woody material to produce steam, which appears to be essential for the selective disintegration of the fibrous material.

The procedure of the invention may be applied generally to natural mixtures or agglomerates of cellular cork material and noncork material. Douglas fir bark, especially the thick bark from mature trees, is the preferred starting material, but other barks which contain substantial amounts of cork may be employed, e.g., suitably selected bark from other firs, pines, spruce, hemlock, beech, maple and various species of oak.

The practice and advantages of the present invention will be further illustrated by the following examples:

#### EXAMPLE 1

Douglas fir bark containing large, prominent veins or layers of cork interspersed with layers of noncork material was employed as the starting material. This bark was representative of thick Douglas fir bark from large, mature trees and was a commercial grade of bark which is in plentiful supply at saw mills in the Douglas fir lumber areas along the Pacific Coast, although the cork content was rather lower than average for Douglas fir bark available at the particular mill. The fibrous material predominated in amount, as is usual. This bark was reduced in size by a chipper to fragments averaging about  $\frac{1}{2}$ " x 1" x  $1\frac{1}{2}$ ".

Approximately 130 pounds of the bark were charged to a "Masonite" gun of the type described above. Steam was introduced until the pressure within the gun rose to 220 p.s.i.g.<sup>1</sup> and was held at that pressure for 30 seconds. Then more steam was admitted until the pressure increased to 600 p.s.i., such step requiring an additional 30 seconds. The outlet port, which in this instance was an opening about 4 inches in diameter, was opened wide. The steam pressure within the gun blew the contents into a commercial drying system normally employed to dry fiberized redwood for another purpose. The effluent from the gun was a very moist, water-laden product. It was dried in the said commercial drying system by countercurrent contact with hot air. A portion of the dried product was separated into different size fractions, as follows:

The dry mass was passed through a  $\frac{3}{8}$ " screen. 55 Oversize ( $+\frac{3}{8}$ ") material was rejected and the  $-\frac{3}{8}$ " material was screened to yield  $-\frac{3}{8}$ " +8, -8 +14, -14 +48, -48 +140, and -140 fractions. These fractions were subjected to physical and chemical tests with results as given in Table I below.

<sup>1</sup> All pressures herein are pounds per square inch gauge.

Table I

| Fraction                            | Product of Example 1 |        |         |          |      | Product of Example 2 |        |         |          |      |
|-------------------------------------|----------------------|--------|---------|----------|------|----------------------|--------|---------|----------|------|
|                                     | $-\frac{3}{8}$ " +8  | -8 +14 | -14 +48 | -48 +140 | -140 | $-\frac{3}{8}$ " +8  | -8 +14 | -14 +48 | -48 +140 | -140 |
| Percent by wt.                      | 29.5                 | 8.9    | 20.9    | 27.1     | 13.6 | 15.3                 | 7.8    | 25.0    | 34.3     | 17.8 |
| pH in dist. water                   | 3.95                 | -----  | 3.85    | 4.0      | 3.85 | 4.1                  | -----  | 3.85    | 4.0      | 3.85 |
| Solub. in hot water, percent by wt. | 8.4                  | -----  | 14.8    | 12.1     | 13.5 | 12.2                 | -----  | 12.1    | 11.0     | 13.2 |
| Solub. in 1% NaOH, percent by wt.   | 59.4                 | -----  | 57.0    | 57.2     | 61.6 | 63.1                 | -----  | 56.1    | 48.3     | 58.2 |
| Solubility in ethyl-alc.            | 21.9                 | -----  | 24.5    | 22.2     | 31.9 | 23.8                 | -----  | 24.4    | 21.3     | 31.3 |
| Bulk density, #/cu. ft.             | 18.1                 | 17.0   | 18.1    | 25.0     | 29.7 | 18.1                 | 17.0   | 18.1    | 25.0     | 29.7 |

## EXAMPLE 2

An equal weight of chips taken from the same lot as Example 1 was charged to the same Masonite gun and was treated in the same manner, except that after bringing the steam pressure in the gun to 600 p.s.i.g., it was held at that pressure for 60 seconds. The contents of the gun were then blown. A similar size classification was effected and similar tests were applied, with results as given in Table I.

It will be apparent that the more severe conditions of Example 2 produced a higher proportion of finer material (-14 mesh) than the less severe conditions of Example 1. It will also be apparent that the finest fractions (-140) yielded the highest percentage of alcohol solubles. It was noted that all of the alcohol extracts precipitated a waxy, amorphous solid on cooling. It was further noted by visual inspection that the  $-\frac{3}{8}'' + 8$  mesh fraction contained particles of cork with fibrous material attached and that the -140 fraction was a black-brown, free-flowing powder.

A further sample of the product of Example 2 was screened to yield  $+\frac{3}{8}''$ ,  $-\frac{3}{8}'' + 8$ ,  $-8 + 14$ ,  $-14 + 48$ ,  $-48 + 140$  and  $-140$  fractions. The coarsest fraction ( $+\frac{3}{8}''$ ) was discarded. A visual inspection was made of the remaining fractions, with the aid of a microscope in the case of the finer fractions. The percentage of cork in each of these fractions was determined with substantial accuracy by hand separation, with results as follows:

Table II.—Cork concentration in various fractions as determined by hand separation

| (1) Fraction                   | $-\frac{3}{8}'' + 8$ | $-8 + 14$ | $-14 + 48$ | $-48 + 140$ | $-140$ |
|--------------------------------|----------------------|-----------|------------|-------------|--------|
| (2) Percent of total bark      | 15.3                 | 7.8       | 25.0       | 34.3        | 17.6   |
| (3) Percent cork in fraction   | 67                   | 63        | 55         | Very small  |        |
| (4) Percent cork in total bark | 10.3                 | 4.9       | 13.8       | Very small  |        |
| (5) Percent of total cork      | 36                   | 17        | 48         | Very small  |        |

Table II requires some explanation. Inspection of the -48 fractions by microscope revealed the presence of cork but in very small quantities and of particle sizes so small that hand separation was not deemed practical. The "percent of total bark" in line (2) excludes the discarded  $+\frac{3}{8}''$  bark. This is considered justified because  $+\frac{3}{8}''$  particles may be considered unprocessed and would be recycled in a continuous commercial process. Also, to some extent, these oversize particles were nonbark contaminants. Line (2), therefore, gives the quantity of each of the size fractions  $-\frac{3}{8}'' + 8$ ,  $-8 + 14$ ,  $-14 + 48$ ,  $-48 + 140$  and  $-140$  expressed as a percentage of the total bark treated after separating the oversize material.

Line (3) gives the quantity of cork in each of the first three fractions, expressed as a percentage of that fraction. The figures in line (4) are arrived at by multiplying each of the figures in line (2) by the corresponding figure in line (3) expressed as a decimal; i.e.,  $15.3 \times 0.67 = 10.3\%$ , etc. Therefore the figures in line (4) represent the quantity of cork in each of the respective fractions, expressed as a percentage of the total bark. Line (5) gives the quantity of cork in each of the first three fractions expressed as a percentage of the total cork in the bark. The figures in line (5) reflect a minor inaccuracy arising from the assumption that no cork existed in the -48 fractions. This inaccuracy was not of great magnitude. Microscopic inspection revealed very little cork in these fractions, and to a considerable extent the cork in these fractions existed as very small particles in the bark of so small a size as to have very limited commercial utility.

It will be seen from Table II that the first two frac-

tions, i.e.,  $-\frac{3}{8}'' + 8$  and  $-8 + 14$ , accounted for  $15.3 + 7.8 = 23.1\%$  of the total bark; that these two fractions contained cork in a concentration of

$$\frac{15.3 \times 67 + 7.8 \times 63}{15.3 + 7.8} = 66\%$$

and that these two fractions contained

$$\frac{10.3 + 4.9}{10.3 + 4.9 + 13.8} \times 100 = 53\%$$

of the total cork in the bark, assuming a negligible quantity of cork in the -48 fractions.

It follows, therefore, that approximately one-half (53%) of the cork in the bark was concentrated in approximately one-quarter (23.1%) of the product consisting of the  $-\frac{3}{8}'' + 8$  and  $-8 + 14$  fractions.

The coarser fractions, particularly the  $-\frac{3}{8}'' + 8$  and  $-8 + 14$  fractions, are commercially useful without further processing. Thus these fractions, although they are not pure cork, are so enriched in cork that they can be used as insulation material in applications which do not require the highest quality of cork. Thus these fractions may be poured loose into an insulating space beneath a floor, above a ceiling or in a wall space. A binder such as resin or asphalt may be employed to bind the particles together. The same fractions may also be used as fillers or extenders for other, more expensive insulating materials such as pure cork from the cork oak.

The finer fractions, such as the  $-48 + 140$  and  $-140$  fractions also have utility, but of a somewhat different type. As mentioned above, by extracting these finer fractions with hot alcohol and cooling the extract, an amorphous waxy solid is produced which is similar to carnauba wax and other waxes of commerce. Also, surface active and dispersing agents can be prepared by extraction with caustic soda or other pulping agents.

It will, therefore, be apparent that the process of the present invention has utility generally as a means of separating cellular, corky material from fibrous and amorphous noncorky material contained in natural mixtures of the two such as Douglas fir bark.

As noted, the coarser fractions are enriched in cork but still contain a considerable proportion of noncork material. Most of the latter in the coarsest fractions ( $-\frac{3}{8}'' + 8$ ) and ( $-8 + 14$ ) is present in the form of fibers and bundles or masses of fibers attached to the cork particles. Some, however, is present as separate fibers and bundles or masses of fibers. I have found that the attached fibers and fiber bundles and masses can be detached and ground, and that the already separated fibers and fiber bundles and masses can be ground by a relatively light milling operation, as by means of ball or hammer milling or merely tumbling the particles and abrading them against one another. By such means, repeated several times if necessary, followed in each instance by size classification, it is possible to produce relatively coarse (+14) and pure (90-95%) cork.

Some further refinement, if carried out by gentle abrasion methods, yields a pure cork of high quality. The yield, of course, may be reduced. In commercial practice one will determine the optimum degree of refinement, suitably balancing the factors of economy and quality. The following example will illustrate the results obtainable by further refinement.

Table III

|          | Material              | Yield, percent | Purity, percent |
|----------|-----------------------|----------------|-----------------|
| (1)----- | $-\frac{3}{8}'' + 14$ | 23.1           | 66              |
| (2)----- | $-\frac{3}{8}'' + 14$ | 6.3            | 80-85           |

Material (1) was the combined  $-\frac{3}{8}'' + 8$  and  $-8 + 14$  material originally produced as described in Example 2

by steaming and blowing bark, drying, separating and rejecting  $+ \frac{3}{8}$ " material and screening the remainder without grinding. Material (2) was prepared by grinding material (1), then screening. The yield figure 23.1% for material (1) is explained above, and is based on the total bark after separating  $+ \frac{3}{8}$ " material. The yield figure 6.3% for material (2) was obtained by multiplying 23.1% by 27.1%, the latter being the percentage of ground material recovered as  $+14$ . The purity figures give the percentage of cork in each material.

It will be apparent from an inspection of Table III that an operator has the option of higher yields and less purity (e.g., a 23.1% yield and 66% purity) or lower yields and greater purity (e.g., a 6.3% yield and 80-85% purity).

The cork products of the invention may be put to many of the uses of cork from the cork oak; e.g., for thermal insulation, sound absorption, vibration damping, etc. The coarser grades of product may be ground to finer grades to produce insulation cork, composition cork, cork flour for linoleums, etc. And, of course, it may be used as a filler and extender material.

It will, therefore, be apparent that a method has been provided of treating natural cork-noncork mixtures such as Douglas fir bark to separate the cork from the noncork material, without serious damage to the cellular character of the cork. Such method is economical and can be carried out with existing commercial equipment presently in use in the lumber and wood products industries. It is versatile in that higher yields with concomitant reduced quality, or better quality with reduced yields can be selected. The recovered cork is purer in quality than the corresponding material from other known processes of cork separation. Also the separated noncork material has commercial value.

We claim:

1. A method of cork recovery from bark containing a substantial proportion of cork which comprises providing the bark in the form of particles, subjecting said particles to the action of steam at an elevated pressure and for a short period of time, then releasing the pressure suddenly, thereby exploding a large proportion of the fiber

masses into smaller fiber bundles and individual fibers, drying the exploded mass of fibers and cork and effecting a size classification of the dried mass to produce coarser fractions enriched in cork and finer fractions poor in cork.

5 2. The method of claim 1 wherein said bark is Douglas fir bark.

3. A method as set forth in claim 1, wherein at least one of the coarser fractions is subjected to a gentle abrading action to further and selectively reduce the particle size of fibrous noncork material in such fraction, and 10 wherein the abraded fraction is then subjected to a further size classification to yield a coarse fraction of higher cork content.

4. A method of treating bark containing a substantial quantity of cork in admixture with fibrous and amorphous noncork material, said method comprising providing the bark in the form of chips, subjecting the chips to the action of steam at a sufficiently high pressure and 15 for a sufficient period of time to soften the chips and loosen the bond between the cork and noncork material and thereby produce a loose mass interspersed with particles of cork when the steam pressure is suddenly released, then releasing the steam pressure suddenly to explode the steam treated chips into a loose, moist mass of cork and noncork material, then drying the loose mass and subjecting it to size separation and recovering 20 at least the  $- \frac{3}{8}$ "  $+14$  mesh fractions.

5. The method of claim 4 wherein said bark is Douglas fir bark.

30 6. The method of claim 4 wherein the chips are subjected to steam at about 600 p.s.i.g. for about 2 minutes.

References Cited in the file of this patent

UNITED STATES PATENTS

|           |          |               |
|-----------|----------|---------------|
| 2,446,551 | Pauley   | Aug. 10, 1948 |
| 2,711,369 | Birdseye | June 21, 1955 |
| 2,736,063 | Heritage | Feb. 28, 1956 |

OTHER REFERENCES

40 Marple: Douglas Fir Bark Utilized as a Filler, from Plastics, August 1947 (pp. 44, 65, 67).